

Nov. 1, 1938.

J. R. CARPENTER

2,135,047

METHOD FOR CUTTING AGATIZED PETRIFIED WOOD

Filed Dec. 19, 1936

2 Sheets-Sheet 1



Fig. 3.



Fig. 2. 16 15



Fig. 1.

Inventor  
J. Ross Carpenter  
by Doug & Haag.

Nov. 1, 1938.

J. R. CARPENTER

2,135,047

METHOD FOR CUTTING AGATIZED PETRIFIED WOOD

Filed Dec. 19, 1936

2 Sheets-Sheet 2



FIG. 7.



FIG. 5.



FIG. 6.

Inventor  
J. Ross Carpenter  
by Orwig & Hague Atty's

## UNITED STATES PATENT OFFICE

2,135,047

METHOD FOR CUTTING AGATIZED  
PETRIFIED WOOD

J. Ross Carpenter, Cheyenne, Wyo.

Application December 19, 1936, Serial No. 116,734

2 Claims. (Cl. 125—16)

My invention relates to the art of cutting agatized petrified wood. This material is very hard, being rated as almost as hard as the diamond. The methods and apparatus heretofore used for this purpose have not been speedy and accurate enough to make this valuable and highly ornamental material available for general use in a commercially practical manner.

The objects of my invention are to provide a method and apparatus for cutting agatized petrified wood at relatively high speed to thereby greatly reduce the cost of forming it into articles of commerce, whereby this material may be made commercially available for many ornamental and useful articles.

A further object is to provide means of simple and inexpensive construction for holding articles of such irregular outline as agatized petrified logs and pieces thereof, firmly in position so that they may be presented to the cutter with great accuracy and cut to any predetermined thickness, and the cutting completed without any movement of the material being cut, and further in this connection to provide means whereby the cutter may be firmly and accurately held in position relative to the material so that the cutter will enter into and cut from a log of agatized petrified wood a relatively thin slab.

A further object is to provide an apparatus of simple and inexpensive construction for use in practicing my improved method of cutting.

In the accompanying drawings, Figure 1 shows a front elevation of a mechanism embodying my invention, the case portion being in section.

Figure 2 shows a longitudinal sectional view on the line 2—2 of Figure 1.

Figure 3 shows a horizontal sectional view on the line 3—3 of Figure 1.

Figure 4 shows a detail view in vertical transverse section of a block of material being cut, and the position of the cutting blade when moving in one direction, shown by solid lines, and when moving in the opposite direction, by dotted lines.

Figure 5 shows a vertical transverse sectional view of the cement block containing the agatized petrified wood and the base for supporting it upon the carriage.

Figure 6 shows a longitudinal sectional view of same, illustrating kerfs cut through the material; and

Figure 7 shows an inverted perspective view of the cement block.

My improved apparatus comprises a main frame 10 having a track 11 thereon. Mounted on

this track is a movable carriage 12 for carrying the material to be cut.

For the purpose of adjustably fixing the carriage 12 in proper position for cutting slabs of the exact thickness desired I have provided upon the top of the frame between the rails of the track, a channel 13 in which is detachably mounted at one end a spacing bar 14 and at the other end a spacing bar 15, which latter bar is adjustably connected to the main frame by the screw 10 16a. Adjacent this spacing bar 14 is a series of spacing blocks 16, each accurately proportioned to the exact width of the various slabs to be made of the material being cut. To readjust the material being cut, one of said spacing blocks 16 is removed from the front of the material and replaced in the rear of the material being cut, thus providing ease and accuracy in the adjustment of the carriage to proper position.

Mounted in the main frame is an upright 20 clamping frame 17 containing a clamping screw 18 and a follower 19 connected with the screw for securely holding the material to be cut upon the carriage and holding the carriage firmly against the track.

On opposite sides of the carriage are the upright cutter guides 20, having slots 21 through which the cutter frame is extended and guided in its reciprocating movement.

The cutter frame 22 is mounted in said slots 30 and is provided with a cutter blade 23 which may be made of cold rolled steel or the like, and which is smooth and of uniform thickness throughout its length. At one end of the cutter frame is a rigid arm 24 which is pivoted to a crank 25. This crank may be operated in any desired manner. When the crank is operated it imparts to the cutter blade a certain movement essential to the successful operation of my improved art of cutting agatized petrified wood. This movement of 40 the cutter blade is as follows: When the crank is at its lower limit of movement, the portion of the blade nearest the crank engages the material being cut, and the other portion of the blade is elevated out of contact with said material, then 45 when the crank is at its upper limit of movement the portion of the cutter blade furthest from the crank engages the material being cut, and the portion nearest the crank is elevated out of contact therewith. This peculiar movement of the 50 blade enables me to practice my improved art of cutting in a rapid manner.

The material to be cut comprises logs and broken pieces of agatized petrified wood of very irregular outline and very difficult to firmly and 55

securely hold in position to be cut. I have provided means of simple and inexpensive character for firmly holding such material in position and for cutting it with great accuracy into the sizes desired.

I provide a mould box 30, shown in Figure 5, into which the material to be cut is placed, then the mould is filled with cement and permitted to set and harden. This mould is provided with 10 grooves 31 in its bottom portion so that the block of cement 32, when removed, is provided with ribs 32a. I then provide a base block 33 formed with grooves shaped to receive and accurately fit the ribs 32a. Then the base block is placed upon 15 the carriage and firmly fixed thereon. When placing the material to be cut within the mould, I carefully measure the position of each piece of material relative to the end of the mould, and make a record thereof. Then when the cutting is 20 being done, I can cut each piece of the material at the desired place to form the kind of articles desired. In Figure 6 the kerf 34 is shown in position for cutting a thin slab from the log 35. In view of the extreme hardness of the agatized petrified wood this operation is very difficult. I have demonstrated, however, in actual practice that when the material to be cut is embedded in a 25 cement block the cutter will enter a log of agatized petrified wood at the angle shown in said figure, 30 thereby enabling me to cause the cutter to enter a log of agatized petrified wood at any desired angle relative to the surface thereof. When cutting broken pieces of the material marked 36, they may be placed in the mould while the 35 cement is being poured, and positioned one above the other, then the cutter may be accurately positioned to cut through all of said broken pieces in one operation, thereby all of them accurately in one dimension, say, for instance, six inches thick. 40 They are finally reduced to the desired dimension other than thickness by succeeding cutting operations in another cement block.

The blade is reciprocated by the crank and is tilted during this reciprocation. Its action is so arranged that during the movement of the blade in one direction, the blade will engage the article at one end of the kerf being formed, and during this movement the other end of the blade which is moving out of the kerf, is tilted to position out 45 of contact with the kerf at the opposite side thereof, and into contact with the kerf at the middle portion thereof, as shown by dotted lines in Figure 4. A similar action takes place in the opposite direction during the return movement of the blade, as shown by solid lines in 50 Figure 4. This movement of the blade accomplishes the following desirable results:

At the ends of the kerf the blade engages only when moving inwardly toward the middle of the 55 material, thus preventing chipping off of particles of the material at those points such as would occur if the blade engaged the ends of the kerf while cutting outwardly. Furthermore, this movement of the blade keeps the liquid carrying the 60 abrasive, hereinafter described, within the kerf for a relatively long time as it continuously moves it from the ends of the kerf toward the center of the material being cut.

The liquid containing the bentonite and the 65 abrasive will flow by gravity from the middle portion of the material being cut because the bottom of the kerf inclines downwardly in both directions from the middle, and the cutter blade continuously tends to move the said liquid toward the 70 middle of the material being cut. By reason of

these two opposing actions the said liquid is contained within the kerf for a relatively long time, and such liquid as flows from the ends of the kerf is returned as hereinafter described.

Beneath the cutter blade I have formed in the 5 frame a sump 26 in which there is mounted a pump 27. A pipe 28 leads from the pump to a point above the kerf to return the liquid to the blade after it has passed into the sump.

In practicing my improved art I first provide a 10 quantity of bentonite and mix it with sufficient water to form a slippery plastic gelatinous mass that resembles soft soap (see Bentonite, its properties, mixing, preparation and utilization, by C. W. Davis and H. C. Vacher, Technical Paper 15 438, Dept. of Commerce, United States of America). I then thoroughly mix with the wetted bentonite a quantity of finely divided carborundum or other abrasive. I have had satisfactory results with 60 mesh carborundum. After said 20 mixing, the carborundum is held in suspension in the bentonite, and I find that due to this suspension I have been able to obtain such satisfactory results. I then, by the operation of the pump, force the liquid into the kerf, thus applying said 25 mixture to the surface of the cutter blade and that portion of the material being cut, and then operate the cutting blade.

When carborundum alone in finely divided condition is placed between the cutting edge of a 30 reciprocating blade and agatized petrified wood, the carborundum rapidly becomes dull and shattered, and cutting proceeds very slowly. However, when my process is employed I find that the cutting proceeds rapidly and that the carborundum 35 and bentonite may be used repeatedly.

I believe that the reason for this apparent phenomenon is as follows: The cutting blade made of cold rolled steel or other similar metal is relatively porous as compared with the agatized 40 petrified wood, and individual abrasive particles or small groups of them brought beneath the blade by the raising and lowering thereof during its reciprocating motion, slide along with the blade and cut away portions of the material. If, 45 however, these particles of carborundum were permanently lodged in the pores of the cutter blade, they would soon become dulled or destroyed. With my improved apparatus, however, the abrasive-charged cutting edge of the blade is continuously 50 being pressed against and removed from the material. When the blade is thus removed, the gelatinous nature of the bentonite causes quantities of it to adhere to the material being cut, and be removed at times from the cutter blade, 55 which results in at times withdrawing the abrasive particles or groups from the pores of the cutter blade, and then when the blade is again pressed or slapped against the material covered with the said liquid, the suspended abrasive particles enter and become temporarily lodged in different pores, presenting different and new surfaces of the material being cut.

I have found in practice that when a given 60 quantity of said mixture is applied to the cutting 65 blade it is gradually reduced in quantity by being drawn out through the ends of the cut by force of gravity. This material may be pumped up and repeatedly re-applied to the cutter blade for a considerable number of times before the carbo- 70 rundum becomes appreciably or extremely fine and the speed of cutting is decreased.

Another advantage of my improved method is that when a cut is completed through the agatized petrified wood, the faces of the material 75

are free from scratches or grooves and present a smooth, finished appearance. This desirable result is attained because, during a cutting operation, the liquid containing the abrasive is at all times present between the sides of the cutter blade and the adjacent sides of the material being cut, and since there is very little lateral pressure of the blade against the sides of the kerf, the action at the sides of the blade is a smoothing, 5 polishing action, as distinguished from the cutting action before described, at the cutting edge of the blade.

To illustrate this action, it is my present practice in actual use with a full sized machine to 15 use a cutting blade until the under surface is worn away to a great extent. I then reverse the blade so that the former cutting edge is uppermost, and then use the blade in that manner until the new cutting edge is worn away to such 20 an extent as to require a new blade. When this occurs at such time as the material is cut say half way through, I insert a new blade of the same size and thickness as the original blade, and find that it functions properly and completes 25 the cut without any appreciable binding in the cut or unevenness in the surfaces of the kerf.

I claim as my invention:

1. The method of cutting kerfs in agatized petrified wood, which consists in providing a thin, 30 smooth blade made of a metal having a degree of porosity greater than that of agatized petrified wood, providing a jelly-like substance containing in suspension therein a quantity of abrasive particles of such size that they will enter and be 35 come lodged in the pores of the blade and will not enter and become lodged in agatized petrified wood, placing a quantity of said jelly-like substance containing said abrasive particles in contact with both the blade and the material to be 40 cut, then reciprocating the blade against the material being cut, thereby causing portions of said abrasive particles to enter and become lodged in the pores of the blade and be carried by the blade in cutting contact with the material being 45 cut and not lodged in the material being cut, to thereby avoid having said abrasive wear away the blade, then at times during the reciprocation of the blade, causing portions of its cutting edge to move away from contact with the material being cut, to thereby cause some of the abrasive particles carried by the blade to 50 adhere to the material being cut, due to the adhesive quality of the said jelly-like substance, and thereby be withdrawn from the pores of the blade and thereafter returning said portions of the blade to contact with the material being cut and the jelly-like substance thereon to thereby cause other particles of said abrasive substance to enter the pores of the blade and present previously unused particles of the abrasive to cutting positions within the pores of the blade and causing said blade during its reciprocation to first move upwardly and toward the center of the material from one side and then upwardly and toward the center of the material from the other side, to thereby carry the jelly-like substance toward the center of the material being cut.

J. ROSS CARPENTER.

material being cut, due to the adhesive quality of the said jelly-like substance, and thereby be withdrawn from the pores of the blade and thereafter returning said portions of the blade to contact with the material being cut and the 5 jelly-like substance thereon to thereby cause other particles of said abrasive substance to enter the pores of the blade and present previously unused particles of the abrasive to cutting positions projecting from the blade.

2. The method of cutting kerfs in agatized petrified wood, which consists in providing a thin, smooth blade made of a metal having a degree of porosity greater than that of agatized petrified wood, providing a jelly-like substance 15 containing in suspension therein a quantity of abrasive particles harder than agatized petrified wood and of such size that they will enter and become lodged in the pores of the blade and will not enter and become lodged in agatized petrified wood, placing a quantity of said abrasive substance in contact with both the blade and the material to be cut, then reciprocating the blade against the material being cut, thereby causing portions of said abrasive particles to enter and 20 become lodged in the pores of the blade and be carried by the blade in cutting contact with the material being cut and not lodged in the material being cut, to thereby avoid having said abrasive wear away the blade, then at times during the 25 reciprocation of the blade, causing portions of its cutting edge to move away from contact with the material being cut, to thereby cause some of the abrasive particles carried by the blade to adhere to the material being cut, due to the adhesive quality of the said jelly-like substance, and thereby be withdrawn from the pores of the blade and thereafter returning said portions of the blade to contact with the material being cut and the jelly-like substance thereon to thereby 30 cause other particles of said abrasive substance to enter the pores of the blade and present previously unused particles of the abrasive to cutting positions within the pores of the blade and causing said blade during its reciprocation to first 35 move upwardly and toward the center of the material from one side and then upwardly and toward the center of the material from the other side, to thereby carry the jelly-like substance toward the center of the material being cut.

J. ROSS CARPENTER.